

# UNITED STATES PATENT OFFICE.

WILLIAM E. MOWREY, OF ST. PAUL, MINNESOTA.

## PRECIOUS-METAL ALLOY.

1,283,264.

Specification of Letters Patent. Patented Oct. 29, 1918.

No Drawing.

Application filed April 15, 1916. Serial No. 91,470.

*To all whom it may concern:*

Be it known that I, WILLIAM E. MOWREY, a citizen of the United States, residing at St. Paul, in the county of Ramsey and State of Minnesota, have invented certain new and useful Improvements in Precious-Metal Alloys, of which the following is a specification.

This invention relates particularly to alloys designed for use as substitutes for platinum in the manufacture of jewelry, scientific instruments, dental supplies, electrical apparatus, etc.

One object of my invention is to provide an alloy which will be cheaper than platinum but shall not be inferior to it for the purposes for which it is designed.

Another object of my invention is to provide a substitute for platinum which with certain percentages of materials used shall possess a color such as will render it indistinguishable from platinum.

Another object of my invention is to provide an alloy as a substitute for platinum that shall be non-oxidizable.

With these and incidental objects in view the invention consists of certain combinations of metals as hereinafter set forth in this specification.

In producing my improved alloy I fuse together palladium, silver and gold, and the proportions of these metals may be varied without departing from my invention, as I believe myself to be the first to produce an alloy of these three metals combined in any proportion.

To produce an alloy for dental work ex-

clusively, I prefer to use 5% of palladium, 45% of silver and 50% of gold. This combination produces a metal that is satisfactory for all dental work, is considerably cheaper than platinum, is easily workable, possesses a tensile strength sufficiently high for the purposes for which it is designed, is capable of receiving a high polish, and has wearing qualities equal to those of platinum.

As an alloy to be used in electrical work, jewelry work, and certain dental work, I prefer a combination of 15% of palladium, 35% of silver, and 50% of gold. This combination is practically indistinguishable from platinum and has all of the qualities needed for the classes of work for which it is designed.

With either of the combinations herein set forth, or in any of the other combinations that may be made within the scope of this invention, the metals are melted together in a crucible with any suitable flux, although I prefer to use as a flux, boracic acid, on account of its cleanliness and purity.

While I have more specifically described two combinations of the three metals, I do not wish it understood that I limit myself to these combinations, as my invention contemplates any mixture of these three metals, as set forth in the following claim.

### Claim:

An alloy for dental, jewelry and electrical purposes, comprising substantially 15 per cent. of palladium, substantially 35 per cent. of silver, and substantially 50 per cent. of gold fused together.

WILLIAM E. MOWREY.